# EUROPEAN PATENT SPECIFICATION

(11) **EP 4 263 882 B1**
(45) Date of publication and mention of the grant of the patent: **01.10.2025**
(21) Application number: 21819985.9
(22) Date of filing: 03.12.2021
(51) Int. Cl.: C21D 1/673, C21D 6/00, C21D 8/02, C21D 9/40, C21D 9/46, C22C 38/02, C22C 38/04, C22C 38/12, C22C 38/38, C23C 2/02, C23C 2/12, C23C 2/26, C23C 2/28, C23C 2/40

(54) **COATED STEEL SHEET AND HIGH STRENGTH PRESS HARDENED STEEL PART AND METHOD OF MANUFACTURING THE SAME**
BESCHICHTETES STAHLBLECH UND HOCHFESTES PRESSGEHÄRTETES STAHLTEIL UND HERSTELLUNGSVERFAHREN DAFÜR
TÔLE D'ACIER REVÊTUE, PIÈCE EN ACIER TREMPÉ SOUS PRESSE À HAUTE RÉSISTANCE ET LEUR PROCÉDÉ DE FABRICATION

(30) Priority: 16.12.2020 WO PCT/IB2020/062045
(43) Date of publication of application: 25.10.2023
(62) Divisional of application: 25197585.0
(73) Proprietor: ArcelorMittal, 1160 Luxembourg (LU)
(72) Inventor: PHILIPPOT, Clément, 57365 Ennery (FR); LE GUILLARD, Sandra, 54800 Mars La Tour (FR); DUSSAUSSOIS, David, 54310 Homécourt (FR); SALIB, Matthieu, 57283 Maizières-lès-Metz Cedex (FR)
(74) Representative: Lavoix
(86) International application number: PCT/IB2021/061291
(87) International publication number: WO 2022/130101

(56) References cited:
- WO-A1-2014/188830
- WO-A1-2017/006159
- WO-A1-2018/220540
- WO-A1-2019/171157
- US-A1- 2017 260 599
- US-A1- 2018 237 877

## Description

The present invention relates to coated steel sheets and to high strength press hardened steel parts having good bendability properties.

High strength press-hardened parts can be used as structural elements in automotive vehicles for anti-intrusion or energy absorption functions.
In such type of applications, it is desirable to produce steel parts that combine high mechanical strength, high impact resistance and good corrosion resistance. Moreover, one of major challenges in the automotive industry is to decrease the weight of vehicles in order to improve their fuel efficiency in view of the global environmental conservation, without neglecting the safety requirements.

This weight reduction can be achieved in particular thanks to the use of steel parts with a martensitic or bainitic/martensitic microstructure.

The publication WO2016104881 relates to a hot press forming part used as a structural part of a vehicle or the like, requiring impact resistance characteristics, and more particularly, having a tensile strength of 1300 MPa or greater and a method for manufacturing the same by heating a steel material to a temperature at which an austenite single phase may be formed, and quenching and hot forming thereof using a mold. To obtain such properties, the base steel sheet comprises a thin ferrite layer lower than 50 µm at the surface, and the carbides size and density should be controlled. This ferrite layer in the substrate allow to inhibit the propagation of the fine cracks formed on the plating layer to the base but leads to a low bendability with bending angle lower than 70°.

The publication WO2018179839 relates to a hot-pressed part obtained by hot pressing a steel sheet having a microstructure changing in the thickness direction, with a soft layer made of at least 90% of ferrite, a transition layer made of ferrite and martensite and a hard layer mainly martensitic and has both high strength and high bendability. To obtain such properties, the cold rolled steel sheet is annealed in an atmosphere with a dew point temperature comprises from 50°C to 90°C, which could be harmful to aluminium alloy coating. Further prior art is described in US2017/260599A1 and WO2018/220540A1.

The purpose of the invention therefore is to solve the above-mentioned problem and to provide a press hardened steel part having a combination of high mechanical properties with the tensile strength TS above or equal to 1500 MPa and bending angle higher than 70°. The the press hardened steel part according to the invention has yield strength YS above or equal to 1250 MPa.

Another purpose of the invention is to obtain a coated steel sheet that can be transformed by hot forming into such a press hardened steel part.

The object of the present invention is achieved by providing a steel sheet according to claim 1. Another object is achieved by providing the method according to claim 2. Another object of the present invention is achieved by providing a press hardened steel part according to claim 3. The steel part can also comprise characteristics of claim 4. Another object is achieved by providing the method according to claim 5.

The invention will now be described in detail and illustrated by examples without introducing limitations, with reference to the appended figures:
- Figure 1a illustrates a schematic section of the coated steel sheet of trial 4, which is not according to the invention
- Figure 1b represents a schematic section of the press hardened steel part from trial 4 which is not according to the invention
- Figure 2a illustrates a schematic section of the coated steel sheet of trial 3, which is not according to the invention
- Figure 2b represents a schematic section of the press hardened steel part from trial 3 which is not according to the invention
- Figure 3a illustrates a schematic section of the coated steel sheet of trial 2, which is according to the invention
- Figure 3b represents a schematic section of the press hardened steel part from trial 2 which is according to the invention
- Figure 4a illustrates a schematic section of the coated steel sheet of trial 1, which is according to the invention
- Figure 4b represents a schematic section of the press hardened steel part from trial 1 which is according to the invention
- Figure 5a illustrates a schematic section of the coated steel sheet of trial 5, which is not according to the invention
- Figure 5b represents a schematic section of the press hardened steel part from trial 5 which is not according to the invention

The composition of the steel according to the invention will now be described, the content being expressed in weight percent.

According to the invention the carbon content is comprised from 0.26% to 0.40 % to ensure a satisfactory strength. Above 0.40% of carbon, weldability and bendability of the steel sheet may be reduced. If the carbon content is lower than 0.26%, the tensile strength will not reach the targeted value.

The manganese content is comprised from 0.5% to 1.8 %. Above 1.8% of addition, the risk of central segregation increases to the detriment of the bendability. Below 0.5% the hardenability of the steel sheet is reduced. Preferably the manganese content is comprised from 0.5% to 1.3%.

According to the invention, silicon content is comprised from 0.1% to 1.25%. Silicon is an element participating in the hardening in solid solution. Silicon is added to limit carbides formation. Above 1.25%, silicon oxides form at the surface, which impairs the coatability of the steel. Moreover, the weldability of the steel sheet may be reduced. Preferably, the silicon content is from 0.2% to 1.25%. More preferably the silicon content is from 0.3% to 1.25%. More preferably, the silicon content is from 0.3% to 1%.

The aluminium content is comprised from 0.01% and 0.1% as it is a very effective element for deoxidizing the steel in the liquid phase during elaboration. Aluminium can protect boron if titanium content is not enough. The aluminium content is lower than 0.1% to avoid oxidation problems and ferrite formation during press hardening. Preferably the aluminium content is comprised from 0.01% to 0.05%.

According to the invention, the chromium content is comprised from 0.1% to 1.0 %. Chromium is an element participating in the hardening in solid solution and must be higher than 0.1%. The chromium content is below 1.0% to limit processability issues and cost.

The titanium content is comprised from 0.01% to 0.1% in order to protect boron from formation of BN. Titanium content is limited to 0.1% to avoid TiN formation.

According to the invention, the boron content is comprised from 0.001% to 0.004%. Boron improves the hardenability of the steel. The boron content is not higher than 0.004% to avoid a risk of breaking the slab during continuous casting.

Some elements can optionally be added.

Nickel may be added as an optional element up to 0.5% as it can substantially reduce the sensitivity to delayed fracture.

Molybdenum content can optionally be added up to 0.40%. As boron, molybdenum improves the hardenability of the steel. Molybdenum is not higher than 0.40% to limit cost.

According to the invention, niobium can optionally be added up to 0.08% to improve ductility of the steel. Above 0.08% of addition, the risk of formation of NbC or Nb(C,N) carbides increases to the detriment of the bendability. Preferably the niobium content is below or equal to 0.05%.

Calcium may be also added as an optional element up to 0.1%. Addition of Ca at the liquid stage makes it possible to create fine oxides which promote castability of continuous casting.

The remainder of the composition of the steel is iron and impurities resulting from the smelting. In this respect, P, S and N at least are considered as residual elements which are unavoidable impurities. Their content is less than 0.010 % for S, less than 0.020 % for P and less than 0.010 % for N.

The microstructure of the coated steel sheet according to the invention will now be described.

A section of a coated steel sheet of the invention is schematically represented on Fig 3a and Fig 4a. The coated steel sheet comprises a bulk (2) topped by a decarburized layer (3) comprising in upper part a ferrite layer having a thickness from 1µm to 100 µm (4), and a coating layer (1). Preferably, the thickness of the ferrite layer is comprised from 20 µm to 100 µm. More preferably, the thickness of the ferrite layer is from 25 µm to 100 µm. More preferably the thickness of the ferrite layer is from 30 µm to 80 µm.

The bulk of the coated steel sheet (2) has a microstructure comprising, in surface fraction, from 60% to 90% of ferrite, the rest being martensite-austenite islands, pearlite or bainite.

This ferrite is formed during the intercritical annealing of the cold rolled steel sheet. The rest of the microstructure is austenite at the end of the soaking, which transform into martensite-austenite islands, pearlite or bainite during the cooling of the steel sheet.

The decarburized layer present on top of the bulk is obtained during the annealing of the cold rolled steel sheet thanks to the control of the atmosphere in the furnace to set a dew point temperature strictly higher than -10°C and below or equal to 20°C.

The coated steel sheet according to the invention can be produced by any appropriate manufacturing method and the man skilled in the art can define one. It is however preferred to use the method according to the invention comprising the following steps:
A semi-product able to be further hot-rolled, is provided with the steel composition described above. The semi product is reheated at a temperature comprised from 1150°C to 1300°C.

The steel sheet is then hot rolled at a finish hot rolling temperature comprised from 800°C to 950°C.

The hot-rolled steel is then cooled and coiled at a temperature T_{coil} lower than 670°C, and optionally pickled to remove oxidation.

The coiled steel sheet is then cold rolled to obtain a cold rolled steel sheet. The cold-rolling reduction ratio is preferably comprised from 20% to 80%. Below 20%, the recrystallization during subsequent heat-treatment is not favored, which may impair the ductility of the steel sheet. Above 80%, there is a risk of edge cracking during cold-rolling.

The steel sheet is then annealed in an HNx atmosphere with from 0% to 15% of H2, to an annealing temperature T_{A} comprised from 700°C to 850°C and maintained at said annealing temperature T_{A} for a holding time t_{A} comprised from 10s to 1200s, in order to obtain an annealed steel sheet.. Below 700°C, the kinetic of formation of the decarburized layer is too slow to obtain a ferrite layer in its upper part. The holding time t_{A} is above or equal to 10 s to allow the ferrite layer to form, and below or equal to 1200s in order to limit the thickness of this ferrite layer.

During this annealing, the atmosphere in the furnace is controlled to have a dew point temperature T_{DP1} strictly higher than -10°C and below or equal to +20°C in order to form a decarburized layer according to the invention. If T_{DP1} is below or equal to -10°C, the formation of the decarburized layer is slowed down and the ferrite layer is not formed in its upper part. The bendability of the steel part will be too low. If T_{DP1} is higher than 20°C, the surface of the steel sheet may be completely oxidized, impairing coatability and mechanical properties of the sheet
In an embodiment of the invention the annealed steel sheet is heated to an annealing temperature T2 comprised from 700°C to 850°C and maintained at said temperature T2 for a holding time t2 comprised from 10s to 1200s, the atmosphere having a dew point T_{DP2} strictly higher than -10°C and below or equal to +20°C.

The steel sheet is then coated with an aluminium alloy coating.

The microstructure of the press hardened steel part according to the invention will now be described. A section of the press hardened steel part is schematically represented on Fig 3b and Fig 4b.

The steel part comprises successively from the bulk to the surface of the steel part:
- a bulk (7) having a microstructure comprising, in surface fraction, more than 95% of martensite and less than 5% of bainite,
- a ferritic interdiffusion layer (6),
- a coating layer (5) based on aluminium.

During the heating of the steel blank cut out of the steel sheet according to the invention, all microstructural elements of the bulk are transformed into austenite, and the ferrite of the decarburized layer is transformed into austenite with wider grain size than the austenite of the bulk. After hot forming, the steel part is then die-quenched. The interdiffusion layer grows from the former wide grain size austenite layer, thus having larger grain width than prior austenitic grain size in the bulk. The ratio between the ferritic grain width in the interdiffusion layer GWᵢₙₜ over prior austenite grain size in the bulk PAGS_{bulk}, satisfies following equation: $\left({GW}_{int}/{PAGS}_{bulk}\right) - 1 \geq 30 %$ in order to improve bendability of the steel sheet, without deteriorating mechanical properties.

The ferritic grain width is the average distance between two parallel grain boundaries of the interdiffusion layer, grain boundaries being oriented in the direction of the thickness of the sheet. The combination of annealing temperature T_{A}, annealing time t_{A} and dew point temperature T_{DP1} according to the invention promotes the formation of large grain width GWᵢₙₜ in the interdiffusion layer. Moreover, the thermal treatment of the steel blank before the press forming, rules the austenitic grain growth and so the PAGS in the bulk.

In an embodiment, the press hardened steel part may further comprise a martensite layer with a carbon gradient between the bulk and the interdiffusion layer, as represented by (8) in Fig 4b. During the heating of the steel blank, carbon diffuses from the bulk to the surface. The ferrite upper part of the decarburized layer is then transformed in a layer of austenite with a gradient of carbon. During the die-quenching, this layer of austenite with a gradient of carbon is transformed in a layer of martensite with a carbon gradient.

The press hardened steel part according to the invention has a tensile strength TS above or equal to 1500 MPa and a bending angle higher than 70°. The bending angle has been determined on press hardened parts according to the method VDA238-100 bending Standard (with normalizing to a thickness of 1.5 mm).

According to the invention, the yield strength YS is above or equal to 1250 MPa. TS and YS are measured according to ISO standard ISO 6892-1.

The press hardened steel part according to the invention can be produced by any appropriate manufacturing method and the man skilled in the art can define one. It is however preferred to use the method according to the invention comprising the following steps:
A coated steel sheet according to the invention is cut to a predetermined shape to obtain a steel blank. The steel blank is then heated to a temperature comprised from 880°C to 950°C during 10s to 900s to obtain a heated steel blank.

The heated blank is then transferred to a forming press before being hot formed and die-quenched.

The invention will be now illustrated by the following examples, which are by no way limitative.

### Example

6 grades, which compositions are gathered in table 1, were cast in semi-products and processed into steel sheets, then steel parts, following the process parameters gathered in table 2.

### Table 1 - Compositions

The tested compositions are gathered in the following table wherein the element contents are expressed in weight percent.

| Steel | C | Mn | Si | Al | Cr | Ti | B | P | S | N | Ni | Mo | Nb |
|---|---|---|---|---|---|---|---|---|---|---|---|---|---|
| A | 0.34 | 0.6 | 0.56 | 0.043 | 0.32 | 0.017 | 0.002 | 0.009 | 0.0018 | 0.0027 | 0.43 | 0.19 | 0.052 |
| B | 0.32 | 0.7 | 0.35 | 0.03 | 0.5 | 0.026 | 0.002 | 0.014 | 0.0022 | 0.0059 | 0.028 | 0.21 | - |
| C | 0.36 | 0.6 | 0.53 | 0.035 | 0.34 | 0.014 | 0.003 | 0.011 | 0.001 | 0.0034 | 0.4 | 0.20 | 0.049 |
| D | 0.33 | 0.6 | 0.53 | 0.028 | 0.33 | 0.013 | 0.003 | 0.013 | 0.001 | 0.0041 | 0.4 | 0.17 | 0.046 |
| E | 0.36 | 1.3 | 0.28 | 0.003 | 0.25 | 0.02 | 0.003 | 0.01 | 0.002 | 0.006 | - | - | - |
| F | 0.21 | 1.2 | 0.27 | 0.018 | 0.15 | 0.037 | 0.002 | 0.01 | 0.002 | 0.006 | 0.012 | - | - |

| | | | | | | | | | | | | | |
|---|---|---|---|---|---|---|---|---|---|---|---|---|---|
| Steels A-D are according to the invention. Underlined values: not corresponding to the invention | | | | | | | | | | | | | |

### Table 2 - Process parameters

Steel semi-products, as cast, were reheated at 1200 °C, hot rolled with a finish hot rolling temperature comprised from 800 to 950°C, coiled at 550°C and cold rolled with a reduction rate of 60%. Steel sheets are then heated to a temperature T_{A} and maintained at said temperature for a holding time t_{A}, in an HNx atmosphere with 5% of H₂, having a controlled dew point. The steel sheets were then cooled down to a temperature from 560 to 700°C and then hot dip coated with an aluminium-silicon coating comprising 10% of silicon.

Samples 1,2,5 and 6 did undergo a second annealing at a temperature T₂ before coating, the steel sheet being maintained at said T₂ temperature for a holding time t₂, in an HNx atmosphere with 5% of H₂ and a controlled dew point. The following specific conditions were applied:

| Trial | Steel | Soaking | | | Second soaking | | |
|---|---|---|---|---|---|---|---|
| | | t_{A} (s) | T_{A} (°C) | T_{DP1} (°C) | t₂ (s) | T₂ (°C) | T_{DP2} (°C) |
| 1 | A | 135 | 850 | 10 | 70 | 800 | 0 |
| 2 | B | 135 | 850 | 10 | 70 | 800 | 0 |
| 3 | C | 240 | 755 | -10 | - | - | - |
| 4 | D | 30 | 730 | -40 | - | - | - |
| 5 | E | 10800 | 700 | 0 | 70 | 750 | 0 |
| 6 | F | 135 | 850 | 10 | 70 | 800 | 0 |

Underlined values: not corresponding to the invention

The coated steel sheets were analyzed, and the corresponding properties of decarburized layer are gathered in table 3.

**Table 3 - Properties of the decarburized layer of the coated steel sheet**

| Trial | Presence of decarburized layer | Thickness of the ferrite upper part of the decarburized layer (µm) |
|---|---|---|
| 1 | yes | 60 |
| 2 | yes | 35 |
| 3 | yes | - |
| 4 | no | - |
| 5 | yes | 140 |
| 6 | yes | 60 |

| | | |
|---|---|---|
| Underlined values: not corresponding to the invention | | |

The coated steel sheets were then cut to obtain a steel blank, heated at 900°C during 6 minutes and hot-formed. The steel parts were analyzed and the corresponding microstructure, ferritic grain width in interdiffusion layer GWᵢₙₜ, and prior austenite grain size in the bulk PAGS_{bulk} are gathered in table 4. Mechanical properties are gathered in Table 5.

**Table 4 - Microstructure of the press hardened steel part**

| Trial | Bulk microstructure | (GWᵢₙₜ / PAGS_{bulk} )-1 | GWᵢₙₜ (µm) | PAGS_{bulk} (µm) |
|---|---|---|---|---|
| 1 | 100% martensite | 83% | 9.9 | 5.4 |
| 2 | 100% martensite | 128% | 16.9 | 7.4 |
| 3 | 100% martensite | 27% | 6.6 | 5.2 |
| 4 | 100% martensite | -2% | 4.9 | 5 |
| 5 | 10% ferrite | | | |
| | 70% bainite | | | |
| | 20% martensite | n.d | 8.3 | n.d |
| 6 | 100% martensite | 45% | 8.9 | 7.8 |

| | | | | |
|---|---|---|---|---|
| Underlined values: not corresponding to the invention n.d: non determined | | | | |

The surface fractions, ferritic grain width in the interdiffusion layer and PAGS are determined through the following method: a specimen is cut from the press hardened steel part, polished and etched with a reagent known per se, to reveal the microstructure. The section is afterwards examined through optical or scanning electron microscope, for example with a Scanning Electron Microscope with a Field Emission Gun ("FEG-SEM") at a magnification greater than 5000x, coupled to a BSE (Back Scattered Electron) device.

**Table 5 - Mechanical properties of the press hardened steel part**

| Mechanical properties of the tested samples were determined and gathered in the following table: | | | |
|---|---|---|---|
| Trial | TS (MPa) | Bending angle at 1.5mm (°) | YS (MPa) |
| 1 | 1691 | 77 | 1361 |
| 2 | 1649 | 73 | 1296 |
| 3 | 1922 | 36 | 1488 |
| 4 | 1917 | 42 | 1527 |
| 5 | 1566 | 34 | 1183 |
| 6 | 1410 | 65 | 1060 |

| | | | |
|---|---|---|---|
| Underlined values: do not match the targeted values | | | |

The examples show that the steel parts according to the invention, namely examples 1-2 are the only one to show all the targeted properties thanks to their specific compositions and microstructures.

Figure 3a represents a schematic section of the coated steel sheet of trial 2. The combination of process parameters of the invention, annealing temperature T_{A}, annealing time t_{A} and dew point temperature T_{DP1} allow to obtain a decarburized layer (3), in which a layer of ferrite is formed in the upper part (4).

The coated steel sheet is then hot formed. Fig 3b represents a schematic section of the press hardened steel part of trial 2.

The grain width of ferrite formed in the interdiffusion layer (5) is a heritage of the pure ferrite layer in which austenite formation takes place during heating, with larger grain size. The interdiffusion layer grows on this large austenite grain size. The grain width of ferrite in the interdiffusion layer (6) is then larger than prior austenite grain size in the bulk (7), leading to good bendability with bending angle higher than 70°.

Figure 4a represents a schematic section of the coated steel sheet of trial 1. The combination of process parameters of the invention, annealing temperature T_{A}, annealing time t_{A} and dew point temperature T_{DP1} allow to obtain a decarburized layer (3), in which a layer of ferrite is formed in the upper part (4), thicker than in trial 1 due to the higher C content.

The coated steel sheet is then hot formed. Fig 4b represents a schematic section of the press hardened steel part of trial 1.

The grain width of ferrite formed in the interdiffusion layer (6) is a heritage of the pure ferrite layer in which austenite formation takes place during heating, with larger grain size. The interdiffusion layer grows on this large austenite grain size . The grain width of ferrite in the interdiffusion layer (6) is then larger than prior austenite grain size in the bulk (7), leading to good bendability with bending angle higher than 70°. Moreover, due to the thick ferrite layer (4) in the coated steel sheet, a layer of martensite with a carbon gradient is formed between the bulk and the interdiffusion layer in the press hardened steel part, leading to tensile strength higher than 1500 MPa.

In trial 3, the coated steel sheet has a decarburized layer, without ferrite layer in its upper part, as represented schematically in Fig 2a. The absence of ferrite layer is due to the low dew point temperature T_{DP1} of -10°C, which slow down the kinetics of the decarburization.

The coated steel sheet is then hot formed. Figure 2b represents a schematic section of the press hardened steel part from trial 3. Due to the absence of the ferrite layer, the ferritic grain width in the interdiffusion layer (6) is then equivalent to prior austenite grain size in the bulk (7), leading to a low bending angle below 70°.

In trial 4, the low dew point temperature T_{DP1} of -40°C implies an absence of the decarburized layer and ferrite layer in the coated steel sheet.

Fig 1a represents a schematic section of the coated steel sheet of this trial, with the coating layer (1) and the bulk (2).

The coated steel sheet is then hot formed. Figure 1b represents a schematic section of the press hardened steel part from trial 4. Due to the absence of the ferrite layer, the ferritic grain width in the interdiffusion layer (6) is then equivalent to prior austenite grain size in the bulk (7), leading to a low bending angle below 70°.

In trial 5, the steel sheet is maintained during 10800s at soaking temperature, which form in the coated steel sheet, a thicker ferrite layer in the decarburized layer than previous trials. Fig 5a represents a schematic section of the coated steel sheet of trial 5, with the coating layer (1) the decarburized layer (3), the thicker ferrite layer (4) with coarser grain size, and the bulk (2).

The coated steel sheet is then hot formed and Fig 5b represents a schematic section of the press hardened steel part from trial 5. During the heating of the steel part, the microstructure of the bulk is austenitic, and the thick ferrite layer is transformed in a layer of austenite with gradient of carbon. But due to the thickness of the ferrite layer higher than 100 µm, a layer of ferrite remains present between the interdiffusion layer and the layer of austenite with gradient of carbon.

During die quenching of the steel part, the ferrite layer is still present and the layer of austenite with carbon gradient transforms into a martensite layer with gradient of carbon, leading to a multi-phased layer. This triggers a decrease of yield strength.

In trial 6, the steel sheet has a low carbon level of 0.21%. This low carbon content combined to the process parameters, leads to a decarburized layer in the coated steel sheet with the ferrite layer. Nevertheless, the yield strength and tensile strength of the press hardened steel part are not achieved because of the low level of carbon.

## Claims

1. A coated steel sheet made of a steel having a composition comprising, by weight percent:
C : 0.26 - 0.40 %
Mn : 0.5 - 1.8 %
Si: 0.1 - 1.25 %
Al : 0.01 - 0.1 %
Cr : 0.1 - 1.0 %
Ti: 0.01 - 0.1 %
B: 0.001 - 0.004 % $P \leq 0.020 %$ $S \leq 0.010 %$ $N \leq 0.010 %$
and comprising optionally one or more of the following elements, by weight percent: $Ni \leq 0.5 %$ $Mo \leq 0.40 %$ $Nb \leq 0.08 %$ $Ca \leq 0.1 %$
the remainder of the composition being iron and unavoidable impurities resulting from the smelting,
said coated steel sheet comprising from the bulk to the surface of the coated steel sheet:
- a bulk with a microstructure comprising, in surface fraction, from 60% to 90% of ferrite, the rest being martensite-austenite islands, pearlite or bainite,
- such bulk being topped by a decarburized layer comprising in upper part a ferrite layer having a thickness from 1µm to 100 µm
- a coating layer made of aluminum or aluminium alloy.

2. A method for producing a coated steel sheet according to claim 1, said method comprising the following successive steps:
- casting a steel to obtain a slab, said steel having a composition according to claim 1,
- reheating the slab at a temperature Tᵣₑₕₑₐₜ comprised from 1100°C to 1300°C,
- hot rolling the reheated slab at a finish hot rolling temperature comprised from 800°C to 950°C
- coiling the hot rolled steel sheet at a coiling temperature T_{coil} lower than 670°C to obtain a coiled steel sheet,
- optionally pickling the coiled steel sheet,
- cold rolling the coiled steel sheet to obtain a cold rolled steel sheet
- Heating the cold rolled steel sheet to an annealing temperature T_{A} comprised from 700°C to 850°C and maintaining the steel sheet at said temperature T_{A} for a holding time t_{A} comprised from 10s to 1200s, to obtain an annealed steel sheet, the atmosphere comprising from 0% to 15% of H2 and having a dew point T_{DP1} strictly higher than -10°C and below or equal to +20°C
- cooling said annealed steel sheet to a temperature range from 560°C to 700°C,
- Coating the annealed steel sheet with aluminium or with an aluminium alloy coating
- Cooling the coated steel sheet to room temperature to obtain a steel sheet having a microstructure according to claim 1.

3. A press hardened steel part, the steel part having a composition comprising, by weight percent:
C : 0.26 - 0.40 %
Mn : 0.5 - 1.8 %
Si: 0.1 - 1.25 %
Al : 0.01 - 0.1 %
Cr : 0.1 - 1.0 %
Ti: 0.01-0.1 %
B: 0.001 - 0.004 % $P \leq 0.020 %$ $S \leq 0.010 %$ $N \leq 0.010 %$
and comprising optionally one or more of the following elements, by weight percent: $Ni \leq 0.5 %$ $Mo \leq 0.40 %$ $Nb \leq 0.08 %$ $Ca \leq 0.1 %$
the remainder of the composition being iron and unavoidable impurities resulting from the smelting,
said steel part comprising successively from the bulk to the surface of the steel part:
- a bulk having a microstructure comprising, in surface fraction, more than 95% of martensite and less than 5% of bainite,
- a ferritic interdiffusion layer,
- a coating layer based on aluminium,
wherein the ratio between the ferritic grain width in said interdiffusion layer GWᵢₙₜ over prior austenite grain size in the bulk PAGS_{bulk}, satisfies the following equation: $\left({GW}_{int}/{PAGS}_{bulk}\right) - 1 \geq 30 %$
and having a tensile strength TS above or equal to 1500 MPa, a yield strength YS above or equal to 1250MPa and a bending angle higher than 70°, TS and YS being measured according to ISO standard ISO 6892-1, and the bending angle according to the method VDA238-100 bending Standard (with normalizing to a thickness of 1.5 mm).

4. A press hardened steel part according to claim 3, wherein the press hardened steel part comprises a layer of martensite with a carbon gradient between said bulk and said ferritic interdiffusion layer.

5. A process for manufacturing a press hardened steel part according to anyone of claims 3 to 4, comprising the following successive steps:
- providing a steel sheet according to claim 1, or produced by a method according to claim 2,
- cutting said steel sheet to a predetermined shape, so as to obtain a steel blank,
- heating the steel blank to a temperature comprised from 880°C to 950°C during 10s to 900s to obtain a heated steel blank,
- transferring the heated blank to a forming press,
- hot-forming the heated blank in the forming press to obtain a formed part,
- die-quenching the formed part

## Patentansprüche

1. Beschichtetes Stahlblech, gefertigt aus einem Stahl, der eine Zusammensetzung aufweist, umfassend in Gewichtsprozent:
C: 0,26-0,40 %
Mn: 0,5-1,8 %
Si: 0,1-1,25 %
Al: 0,01-0,1 %
Cr: 0,1-1,0 %
Ti: 0,01-0,1 %
B: 0,001-0,004 % $P \leq 0 , 020 %$ $S \leq 0 , 010 %$ $N \leq 0 , 010 %$
und optional umfassend eines oder mehrere der folgenden Elemente in Gewichtsprozent: $Mo \leq 0 , 40 %$ $Nb \leq 0,08 %$ $Ca \leq 0,1 %$
wobei der Rest der Zusammensetzung aus Eisen und unvermeidlichen Verunreinigungen besteht, die aus dem Schmelzen resultieren,
das beschichtete Stahlblech umfassend von der Masse bis zur Oberfläche des beschichteten Stahlblechs:
- eine Masse mit einer Mikrostruktur, umfassend in Oberflächenfraktion 60 % bis 90 % Ferrit, wobei der Rest Martensit-Austenit-Inseln, Perlit oder Bainit ist,
- wobei diese Masse durch eine entkohlte Schicht bedeckt ist, umfassend in dem oberen Teil eine Ferritschicht, die eine Stärke von 1 µm bis 100 µm aufweist
- eine Beschichtungsschicht, die aus Aluminium oder einer Aluminiumlegierung gefertigt ist.

2. Verfahren zum Herstellen eines beschichteten Stahlblechs nach Anspruch 1, das Verfahren umfassend die folgenden aufeinanderfolgenden Schritte:
- Gießen eines Stahls, um eine Bramme zu erlangen, wobei der Stahl eine Zusammensetzung nach Anspruch 1 aufweist,
- Wiedererhitzen der Bramme bei einer Temperatur T_{wiedererhitzen} von 1100 °C bis 1300 °C, Warmwalzen der wiedererwärmten Bramme bei einer Fertigwarmwalztemperatur von 800 °C bis 950 °C
- Wickeln des warmgewalzten Stahlblechs bei einer Wickeltemperatur T_{wickel} von weniger als 670 °C, um ein gewickeltes Stahlblech zu erlangen,
- optional Beizen des gewickelten Stahlblechs,
- Kaltwalzen des gewickelten Stahlblechs, um ein kaltgewalztes Stahlblech zu erlangen
- Erhitzen des kaltgewalzten Stahlblechs auf eine Glühtemperatur T_{A} von 700 °C bis 850 °C und Halten des Stahlblechs auf dieser Temperatur T_{A} während einer Haltezeit t_{A} von 10 Sek bis 1200 Sek, um ein geglühtes Stahlblech zu erlangen, die Atmosphäre umfassend 0 % bis 15 % H2 und sie weist eine Taupunkt T_{DP1} von streng über -10 °C und unter oder gleich +20 °C auf
- Abkühlen des geglühten Stahlblechs auf einen Temperaturbereich von 560 °C bis 700 °C,
- Beschichten des geglühten Stahlblechs mit Aluminium oder mit einer Aluminiumlegierungsbeschichtung
- Abkühlen des beschichteten Stahlblechs auf Raumtemperatur, um ein Stahlblech mit einem Mikrostruktur gemäß Anspruch 1 zu erhalten.

3. Pressgehärtetes Stahlteil, wobei das Stahlteil eine Zusammensetzung aufweist, umfassend
in Gewichtsprozent:
C: 0,26-0,40 %
Mn: 0,5-1,8 %
Si: 0,1-1,25 %
Al: 0,01-0,1 %
Cr: 0,1-1,0 %
Ti: 0,01-0,1 %
B: 0,001-0,004 % $P \leq 0,020 %$ $S \leq 0,010 %$ $N \leq 0 , 010 %$
und optional umfassend eines oder mehrerer der folgenden Elemente in Gewichtsprozent: $Mo \leq 0,40 %$ $Nb \leq 0,08 %$ $Ca \leq 0,1 %$
wobei der Rest der Zusammensetzung aus Eisen und unvermeidlichen Verunreinigungen besteht, die aus dem Schmelzen resultieren,
das Stahlteil umfassend nacheinander von der Masse bis zur Oberfläche des Stahlteils:
- eine Masse, die eine Mikrostruktur aufweist, umfassend mehr als 95 % Martensit und weniger als 5 % Bainit,
- eine ferritische Interdiffusionsschicht,
- eine Beschichtungsschicht auf Aluminiumbasis,
wobei das Verhältnis zwischen der ferritischen Kornbreite in der Interdiffusionsschicht GWᵢₙₜ und der vorherigen Austenitkorngröße in der PAGSₘₐₛₛₑ die folgende Gleichung erfüllt: $\left({GW}_{int}/{PAGS}_{masse}\right) - 1 \geq 30 %$
und mit einer Zugfestigkeit TS von mindestens 1500 MPa, einer Streckgrenze YS von mindestens 1250 MPa und einem Biegewinkel von mehr als 70°, wobei TS und YS gemäß der ISO-Norm ISO 6892-1 gemessen werden, und der Biegewinkel gemäß dem Verfahren der Norm VDA238-100 Biegung Standard (mit Normierung auf eine Stärke von 1,5 mm) gemessen wird.

4. Pressgehärtetes Stahlteil nach Anspruch 3, wobei das pressgehärtete Stahlteil eine Martensitschicht mit einem Kohlenstoffgradienten zwischen der Masse und der ferritischen Interdiffusionsschicht umfasst.

5. Verfahren zum Herstellen eines pressgehärteten Stahlteils nach einem der Ansprüche 3 bis 4, umfassend die folgenden aufeinanderfolgenden Schritte:
- Bereitstellen eines Stahlblechs gemäß Anspruch 1 oder durch ein Verfahren gemäß Anspruch 2 hergestellt wird,
- Schneiden des Stahlblechs in eine bestimmte Form, um einen Stahlrohling zu erlangen,
- Erhitzen des Stahlrohlings auf eine Temperatur von 880 °C bis 950 °C für 10 bis 900 Sekunden, um einen erhitzten Stahlrohling zu erlangen,
- Überführen des erhitzten Rohlings an eine Umformpresse,
- Warmumformen des erwärmten Rohlings in der Umformpresse, um ein Formteil zu erlangen,
- Abschrecken des geformten Teils.

## Revendications

1. Tôle d'acier revêtue constituée d'un acier ayant une composition comprenant, en pourcentage en poids :
C : 0,26-0,40 %
Mn : 0,5-1,8 %
Si : 0,1-1,25 %
AI : 0,01-0,1 %
Cr : 0,1-1,0 %
Ti : 0,01-0,1 %
B : 0,001-0,004 % $P \leq 0 , 020 % ,$ $S \leq 0 , 010 %$ $N \leq 0 , 010 % ,$
et comprenant éventuellement un ou plusieurs des éléments suivants, en pourcentage en poids : $Ni \leq 0 , 5 %$ $Mo \leq 0 , 40 %$ $Nb \leq 0 , 08 %$ $Ca \leq 0 , 1 %$
le reste de la composition étant du fer et des impuretés inévitables résultant de la fusion,
ladite tôle d'acier revêtue comprenant de la masse à la surface de la tôle d'acier revêtue :
- une masse avec une microstructure comprenant, en fraction de surface, de 60 % à 90 % de ferrite, le reste étant des îlots de martensite-austénite, de la perlite ou de la bainite,
- une telle masse étant surmontée par une couche décarburée comprenant dans la partie supérieure une couche de ferrite ayant une épaisseur de 1 µm à 100 µm
- une couche de revêtement constituée d'aluminium ou d'alliage d'aluminium.

2. Procédé de production d'une tôle d'acier revêtue selon la revendication 1, ledit procédé comprenant les étapes successives suivantes :
- coulage d'un acier pour obtenir une brame, ledit acier ayant une composition selon la revendication 1,
- réchauffage de la brame à une température T_{réchauffage} comprise entre 1100 °C et 1300 °C,
- laminage à chaud de la brame réchauffée à une température de laminage à chaud de finition comprise entre 800 °C et 950 °C
- enroulement de la tôle d'acier laminée à chaud à une température d'enroulement Tₑₙᵣₒᵤₗₑₘₑₙₜ inférieure à 670 °C pour obtenir une tôle d'acier enroulée,
- décapage chimique éventuel de la tôle d'acier enroulée,
- laminage à froid de la tôle d'acier enroulée pour obtenir une tôle d'acier laminée à froid
- chauffage de la tôle d'acier laminée à froid à une température de recuit T_{A} comprise entre 700 °C et 850 °C et maintien de la tôle d'acier à ladite température T_{A} pendant un temps de maintien t_{A} compris entre 10 s et 1200 s, pour obtenir une tôle d'acier recuite, l'atmosphère comprenant de 0 % à 15 % de H2 et ayant un point de rosée T_{DP1} strictement supérieur à -10 °C et inférieur ou égal à +20 °C
- refroidissement de ladite tôle d'acier recuite à une plage de températures de 560 °C à 700 °C,
- revêtement de la tôle d'acier recuite avec de l'aluminium ou avec un revêtement d'alliage d'aluminium
- refroidissement de la tôle d'acier revêtue à température ambiante pour obtenir une tôle d'acier ayant une microstructure selon la revendication 1.

3. Pièce en acier trempé sous presse, la pièce en acier ayant une composition comprenant, en pourcentage en poids :
C : 0,26-0,40 %
Mn : 0,5-1,8 %
Si : 0,1-1,25 %
Al : 0,01-0,1 %
Cr : 0,1-1,0 %
Ti : 0,01-0,1 %
B : 0,001-0,004 % $P \leq 0 , 020 % ,$ $S \leq 0 , 010 %$ $N \leq 0 , 010 %$
et comprenant éventuellement un ou plusieurs des éléments suivants, en pourcentage en poids : $Ni \leq 0 , 5 %$ $Mo \leq 0 , 40 %$ $Nb \leq 0 , 08 %$ $Ca \leq 0 , 1 %$
le reste de la composition étant du fer et des impuretés inévitables résultant de la fusion,
ladite pièce d'acier comprenant successivement de la masse à la surface de la pièce d'acier :
- une masse ayant une microstructure comprenant, en fraction de surface, plus de 95 % de martensite et moins de 5 % de bainite,
- une couche d'interdiffusion ferritique,
- une couche de revêtement à base d'aluminium,
dans laquelle le rapport entre la largeur de grain ferritique dans ladite couche d'interdiffusion GWᵢₙₜ à la taille de grain d'austénite antérieure dans la masse PAGSₘₐₛₛₑ satisfait l'équation suivante : $\left({GW}_{int}/{PAGS}_{masse}\right) - 1 \geq 30 %$
et ayant une résistance à la traction TS supérieure ou égale à 1500 MPa, une limite d'élasticité YS supérieure ou égale à 1250MPa et un angle de cintrage supérieur à 70°, TS et YS étant mesurés selon la norme ISO 6892-1, et l'angle de cintrage selon la norme de cintrage du procédé VDA238-100 (avec normalisation à une épaisseur de 1,5 mm).

4. Pièce en acier trempé sous presse selon la revendication 3, dans laquelle la pièce en acier trempé sous presse comprend une couche de martensite avec un gradient de carbone entre ladite masse et ladite couche d'interdiffusion ferritique.

5. Processus de fabrication d'une pièce en acier trempé sous presse selon l'une quelconque des revendications 3 à 4, comprenant les étapes successives suivantes :
- fourniture d'une tôle d'acier selon la revendication 1, ou produite au moyen d'un procédé selon la revendication 2,
- découpe de ladite tôle d'acier selon une forme prédéterminée, de sorte à obtenir une ébauche d'acier,
- chauffage de l'ébauche d'acier à une température comprise entre 880 °C et 950 °C pendant 10 s à 900 s pour obtenir une ébauche d'acier chauffée,
- transfert de l'ébauche chauffée vers une presse de formage,
- formage à chaud de l'ébauche chauffée dans la presse de formage pour obtenir une pièce formée,
- trempe en matrice de la pièce formée.
